# EUROPEAN PATENT SPECIFICATION

(11) **EP 1 637 241 B1**
(45) Date of publication and mention of the grant of the patent: **12.09.2012**
(21) Application number: 04734124.3
(22) Date of filing: 20.05.2004
(51) Int. Cl.: B21B 1/02, C22C 38/18, C22C 38/00

(54) **METHOD OF MANUFACTURING A SEAMLESS STEEL PIPE USING AN FE- CR- ALLOY**
VERFAHREN ZUR HERSTELLUNG EINES NAHTLOSEN ROHRES AUS EINER FE- CR- LEGIERUNG
PROCEDE DE FABRICATION D' UN TUBE SANS SOUDURE D'UN ALLIAGE FE- CR

(30) Priority: 22.05.2003 JP 2003144557
(43) Date of publication of application: 22.03.2006
(73) Proprietor: SUMITOMO METAL INDUSTRIES, LTD., Osaka-shi, Osaka 541-0041 (JP)
(72) Inventor: HIDAKA, Yasuyoshi, Osaka 5410041 (JP); ANRAKU, Toshiro, Osaka 5410041 (JP); YAMAKAWA, Tomio, Osaka 5410041 (JP); KITAMURA, Yasufumi, Osaka 5410041 (JP)
(74) Representative: Simons, Amanda Louise
(86) International application number: PCT/JP2004/007223
(87) International publication number: WO 2004/103589

(56) References cited:
- JP-A- 5 228 507
- JP-A- 6 100 931
- JP-A- 6 306 455
- JP-A- 7 178 420
- JP-A- 7 204 703
- JP-A- 8 174 034
- JP-A- 11 342 404

## Description

The present invention relates to a method of manufacturing a seamless steel pipe using an iron base alloy (in the specification simply referred to as "Fe-Cr alloy") billet containing Cr in the range of 5 to 17 %, in more detail, a method that can largely reduce the surface treatment of a billet before manufacturing of seamless steel pipes by blooming.

### BACKGROUND ART

In recent years, for use in oil wells and chemical industries, a demand for steel pipes made of a Fe-Cr alloy is high, and in order to manufacture it efficiently with high quality, the production according to a hot seamless steel pipe manufacturing method is increasing. However, in the manufacture of the Fe-Cr alloy seamless steel pipes, on an external surface of an obtained steel pipe, in some cases, surface defects such as scale flaws are generated.

Such surface defects, in many cases, are caused owing to scale defects on a billet surface prior to tube-making. That is, owing to descaling failure in a manufacturing process of a billet, scales are left without being removed, the scales are squeezed in or rolled together to be the scale defects, and when the billet is subjected to tube-making with the scale defects remained thereon, the surface defects are caused.

Accordingly, an improvement in a method of descaling in the manufacturing process of billet is forwarded. However, at present time, it is difficult to assuredly remove scale residue. Accordingly, in order to prevent the surface defects from occurring on a steel pipe after hot tube-making, almost all the billets are subjected to a surface inspection before tube-making, and based on the results, the surface treatment is applied.

Normally, a billet used for manufacturing the Fe-Cr alloy seamless steel pipe is, as shown in Figs. 1 and 2 that are described later, manufactured by blooming a steel ingot made of the same alloy. The steel ingot after being heated to substantially 1200 °C, is processed by the blooming by means of a box type or grooved roll. At that time, with a multi-stage roll, while gradually reducing it and making a diameter of the material smaller, the steel ingot is finished into a billet shape.

In the blooming, in order to remove the scales generated on the steel ingot owing to heating, the descaling with high-pressure water is applied. However, frequently, a descaling failure is caused, remaining scales are squeezed in or rolled together with a surface of the steel ingot and thereby the scale defects are caused on the surface of the billet.

In order to reduce the scale defects, descaling capability, for instance, an increase in a flow rate and ejection pressure of descaling water is enhanced. However, since as the descaling proceeds, a temperature of a bulk material becomes lower, the manufacture of the billet itself is disturbed, that is, also in the enhancement of the descaling capability, there is a limit. From these situations, at present time, it is difficult to assuredly remove the scale residue on the surface of the billet.

In order to cope with the above problems, there have been proposed various countermeasures of heating equipment. Japanese Patent Application Publication No. 07-258740 proposes, a continuous heating method characterized in that when the steel ingot such as a slab or billet is continuously heated with a combustion burner, the generation of oxidation scale is suppressed during heating, the steel ingot after the heating is oxidized to generate scales excellent in peelability, and thereby surface defects are removed. However, when the proposed method is applied, a large-scale improvement and remodeling of a continuous heating furnace become necessary.

Furthermore, in Japanese Patent Application Publication No.57-2831, a method in which before the blooming, SiC is coated to impart oxidizability and thereby to improve the peelability of the scales is disclosed. However, according to the method disclosed here, coating equipment to coat SiC becomes necessary. Furthermore, the coating operation becomes an off-line operation, resulting in lowering the production efficiency.

Accordingly, either of the countermeasures proposed in Japanese Patent Application Publication Nos. 07-258740 and 57-2831 cannot be brought into actual operation as they are, and also from the capability thereof viewpoint, the complete descaling is difficult. Accordingly, after the manufacture of the billet, the surface treatment prior to tube-making has not yet been omitted.

As a method of surface treatment of the billet before tube-making, there is a conventional method in which flaws are detected by ultrasonic defect detection or the like and portions in concern are externally ground by use of a grinder or a peeler. However, since locations where the flaws occur and the frequency thereof are different from one billet to another billet, automated operation is difficult; as a result, the surface treatment before tube-making normally becomes an off-line operation. Accordingly, the manufacture of the seamless steel pipes from the billet is low in the production efficiency and a work environment of the billet treatment is bad.

In the case of the treatment of the billet being automated, irrespective of locations and rate of incidence of flaws, in some cases, whether flaws are present or not, it is necessary to uniformly grind all billet surfaces to remove and treat. In this case, the yield of the billet is remarkably deteriorated.

In place of the uniform grinding of the surface of the billet like this, as to an automated treatment that specifies positions of flaws, for instance, Japanese Patent Application Publication No. 10-277912 proposes a method of treating surface flaws characterized in that after marking on a steel ingot, image data thereof is collected, and from the image data, surface flaw data is extracted. However, according to the proposed method of treating surface flaws, a lot of equipment and expenses are necessary; accordingly, it is not suitable for a method of treating the billet.

As mentioned above, in manufacturing the billet for use in the manufacture of the seamless steel pipe, in order to prevent the scale defect from occurring on the surface thereof, various proposals have been submitted. However, the complete descaling is difficult, that is, the surface treatment after the manufacture of the billet has not yet been omitted.

Furthermore, in surface treatment of the billet, the operation is usually performed off-line, the production efficiency is low and work environment is bad. Even when the treatment is automated, the production yield is lowered and huge equipment expense is necessary.

Accordingly, a manufacturing method that can omit or reduce the surface treatment of the billet, in particular, a manufacturing method that can largely reduce the surface treatment of the billet after blooming for use in the manufacture of Fe-Cr alloy seamless steel pipes is demanded to be developed.

JP08-174034 discusses a method of manufacturing stainless steel sheet wherein the surface of the slab is shot with blasting material through the blasting treatment and part of the blasting material is left therein before the ferritic stainless steel slab is charged in a slab heating furnace in order to easily form a uniform and thick scale during the slab heating. Hot rolling is carried out thereafter.

JP06-306456 relates to a method of manufacturing ferritic stainless steel sheet with few surface defects by applying shot blasting treatment to a continuously cast slab of ferritic stainless steel, charging this cast slab into a heating furnace in order to generate a scale having uniform thickness and then carrying out hot rolling.

JP11-342404 relates to a method of hot rolling a stainless steel ingot wherein before heating in a heating furnace, one or two compounds selected from calcium compounds and barium compounds and an agent which adheres the compound to the stainless steel surface are applied.

JP07-178420 relates to a method of hot rolling stainless steel slabs which involves soaking and holding the steel slabs in a temperature range of 1000 to 100°C for one to three hours, and then holding the slabs in a temperature range of from 150 to 1520°C, for two or more hours prior to hot rolling in order to reduce scale flaws generated during the hot rolling process.

JP07-204703 relates to a method for generating thin oxide scale of 1 to 7 micron in thickness prior to passing the steel through the finish stands in the temperature range of 950°C or less.

### SUMMARY OF THE INVENTION

The present invention is carried out in accordance with the abovementioned problems of conventional technologies and a demand for development of a manufacturing method, and intends to provide a method that can largely reduce the treatment of the billets before tube-making in the case of seamless steel pipe, being manufactured from a Fe-Cr alloy steel ingot by means of blooming.

In view of the fact that the descaling methods that have been used and proposed so far cannot completely remove the scale defects generated on a surface of the billet, the present inventors hit on an idea of not removing the scales, but positively covering the billet surface with the scale, thereby suppressing the surface defects.

Therefore, the blooming of the steel ingot adopted in the process of manufacturing the Fe-Cr alloy billet was studied in detail.

Figs. 1(a) through 1(c) are diagrams for explaining a blooming process of the steel ingot in a manufacturing process of the billet, and situations of change in cross section of the steel ingot accompanying the blooming process. Fig. 1(a) shows a cross section of the steel ingot before the blooming, Fig. 1(b) showing a cross section of the steel ingot in the middle process of the blooming, and Fig.1(c) showing a cross section of the billet after the blooming. The blooming is performed at both first and second stand. In the first stand, with a grooved roll, for instance, a box type roll and in the second stand with a grooved roll, reverse rolling is respectively carried out.

A steel ingot 1 in the blooming, after being heated to substantially 1200 °C, is gradually reduced for every reduction surface at the first stand. As shown in Fig. 1(b), it is processed into the steel ingot 1 having a rectangular cross section. In the next place, the steel ingot 1 having a rectangular cross section is charged at the second stand, rolled so as to gradually make the cross section smaller and, as shown in Fig. 1(c), finished in a shape like a final billet 2.

Fig. 2 is a diagram of one example for explaining in detail situations of change in a shape of the cross section of the steel ingot in the blooming process in the manufacture of the billet. In the blooming process shown in Fig. 2, the cross section of the steel ingot 1 is gradually reduced and finally finished to a billet 2 after rolling ten passes. In the rolling process, the steel ingot 1 before the blooming is placed so as being laid on the shorter side (corresponding to Fig. 1(a)), and processed so as to be the steel ingot 1 having a rectangular cross section after the rolling of a seven pass at the first stand (corresponding to Fig. 1(b)). Next, the steel ingot having the rectangular cross section is subjected to the eighth through tenth rolling at the second stand and finished into the final billet 2 (corresponding to Fig. 1(c)).

In a page shown in Fig. 2, the first, second, fourth, sixth, eighth and tenth passes show the rolling in the vertical reduction direction, and the third, fifth, seventh and ninth passes show the rolling in the horizontal reduction direction. In an actual rolling, the steel ingot is rotated 90° to change a rolling reduction direction.

The steel ingot 1 shown in Fig. 1(a) is divided into a high reduction rate surface 3 and a low reduction rate surface 4, the high reduction rate surface 3 showing a surface that becomes higher in the reduction rate in the blooming, the low reduction rate surface 4 showing other surface thereof. In the ordinary blooming, as shown in Fig. 2, the steel ingot before the blooming is disposed in the longitudinal direction; accordingly, the high reduction rate surface 3 becomes a surface of shorter side in the slab-shaped steel ingot, the low reduction rate surface 4 becoming a surface of longer side.

However, when by the blooming process shown in Figs. 1(a) through 1(c) and Fig. 2, the steel ingot 1 is reduced for every reducing surfaces at the first stand and further rolled at the second stand to be finished into the billet 2, and, in an external surface of the billet 2, an area ratio of a portion that was the high reduction rate surface 3 to a portion that was the low reduction rate surface 4 in the steel ingot 1 becomes almost the same.

That is, a cross section of the billet 2 after the blooming shown in Fig. 1(c) is equally divided into four portions of two high reduction rate surfaces 3' (portion reduced with high reduction rate of the steel ingot 1) and two low reduction rate surfaces 4' (portion reduced with low reduction rate of the steel ingot 1) and a central angle θ (an angle occupying in a surface portion of the billet 2) of the high reduction rate surface 3' shown in the same drawing becomes 90°.

Fig. 3 is a perspective view showing an entire configuration of the billet after the blooming. In the rolling with the grooved roll at the first stand, a center portion of the low reduction rate surface 4 is not directly restrained by a reduction roll, or, even when restrained, is only slightly restrained compared to other portions. Accordingly, in the billet 2 after the blooming, as shown in Fig. 3, wrinkles 5 are generated in the longitudinal direction of the billet.

As the grooved roll that is used in the blooming, a box type roll, a diamond type roll or an oval type roll can be illustrated. However, the box type roll is effective in preventing the steel ingot from inclining/falling. Accordingly, in view of the stability of the blooming, the box type roll is adopted in many cases.

Accordingly, on the basis of the wrinkles 5 of the billet 2 after the blooming, the high reduction rate surface 3' can be specified in a range of a central angle of ± 45° (θ/2) with a surface h that is orthogonal to the wrinkles 5 as a center of the billet 2.

Based on the knowledge of the high reduction rate surface of the steel ingot and the billet, the manufacturing process of the Fe-Cr alloy billet was further studied in more detail and the following findings (a) through (e) were obtained.
(a) In order to prevent the scale defects from occurring on the surface of the Fe-Cr alloy billet, it is difficult to completely remove the scales generated on the steel ingot before the blooming.
(b) Complete removal of the scales generated on the steel ingot was given up and generation pattern of the scales which are unlikely to be squeezed in or rolled together during the blooming was studied. As a result, scales generated and adhered to the steel ingot over a large covering area were found unlikely to be squeezed in or rolled together during the blooming.
(c) Specifically, in the process of manufacturing the billet, there is no need for descaling with a high-pressure water descaler.
(d) Furthermore, as the rolling of a first pass in the blooming (first stand) is begun from the high reduction rate surface of the steel ingot, the generated scales can be more closely adhered to the steel ingot.
(e) Still furthermore, as heating conditions (atmosphere, heating temperature and holding time) of the steel ingot were adjusted, the scales are unlikely to exfoliate during the blooming and can be generated over a larger covering area of the steel ingot.

The present invention was achieved based on the above findings and a method of manufacturing a seamless pipe using an Fe-Cr alloy billet according to (1) through (3) below are the gist of the invention.
(1) A method of manufacturing a seamless steel pipe, comprising subjecting a steel ingot to blooming to manufacture an Fe-Cr alloy billet wherein the ingot is heated prior to blooming to generate a scale on its surface and wherein blooming is applied without applying descaling of the steel ingot, and manufacturing the seamless steel pipe from the Fe-Cr alloy billet.
(2) A manufacturing method as set out in (1) above, wherein a scale having a thickness of 1000 µm or more is formed on the steel ingot.
(3) In the manufacturing method according to (2), it is preferable to firstly reduce the high reduction rate surface of the steel ingot. Furthermore, the steel ingot is preferably held in an atmosphere containing 2.5 % by volume or more of steam, and at a temperature of 1200 °C or more for 2 hr or more to generate the scale.

In the present invention, the "Fe-Cr alloy" means an iron base alloy containing 5 to 17 % of Cr and, whereby necessary, other alloy elements such as Ni and Mo may be contained.

The "high reduction rate surface" according to the invention means, in the steel ingot, a surface where when the blooming is applied to form into a billet shape, the reduction rate becomes higher, and, in the billet, a portion that was the high reduction rate surface in the steel ingot before the rolling. Normally, in the steel ingot having a slab shape, the high reduction rate surface becomes a shorter side surface.

The "high reduction rate surface" in the billet, as shown in Fig. 3, simply on the basis of the wrinkles, can be specified in a range where a central angle is ± 45° (θ/2) with a central surface orthogonal to the wrinkles with respect to a center of the billet. In order to more accurately specify the "high reduction rate surface" in the billet, results of macro-observation of a cross section of the billet can be used.

Fig. 4 is a diagram showing one example of observation results of macro-photographs of the billet cross section. In the center portion of the macro-observation, as shown with an elliptic of dotted line, segregation correlated with a direction of the cross section of the steel ingot before the blooming can be observed. That is, since a position where the segregation occurs coincides with a final solidifying position of the steel ingot the final solidifying position depends on a shape of cross section made of a longer side surface 4 and a shorter side surface 3 of the steel ingot.

From the observation results of the macro-photograph of the cross section shown in Fig. 4, a surface approximately in parallel with the elliptic of dotted line is the longer side surface 4, the "lower reduction rate surface", and a surface orthogonal to the elliptic of dotted line is the shorter side surface 3, the "higher reduction rate surface". Accordingly, since, in the billet, even after the rolling, the segregation correlated with a direction of cross section of the steel ingot before the blooming remains, from a distribution of the segregation shown by the elliptic dotted line, the "high reduction rate surface" in the billet can be specified.

As mentioned above, the area ratios of the high reduction rate surface and the low reduction rate surface on an external surface of the billet after the manufacture become almost the same, and the cross section of the billet is equally divided into four portions of two high reduction rate surfaces and two low reduction surfaces. Accordingly, a value of an "area rate of the high reduction rate surface" (a ratio of area of scales in the high reduction rate surface) stipulated according to the invention, when multiplied by 1/2, can be replaced by a "total area rate (of billet)" (a ratio of area of scales in an entire area of the billet).

That is, in the invention, "70 % or more in the area rate of the high reduction rate surface" can be stipulated in other words as "35 % or more of total area rate", "80 % or more in the area rate of the high reduction rate surface" can be stipulated in other words as "40 % or more of total area rate", and "90 % or more in the area rate of the high reduction rate surface" can be stipulated in other words as "45 % or more of total area rate".

### BRIEF DESCRIPTION OF THE DRAWINGS

Figs 1(a) through 1(c) are diagrams for explaining a blooming process of a steel ingot a manufacturing step of a billet, and situations of a change in a cross section of the steel ingot accompanying therewith.
Fig. 2 is a diagram of one example for explaining in detail situations of a change in a shape of the cross section of the steel ingot in the blooming process in manufacture of the billet.
Fig. 3 is a perspective view showing an entire constitution of the billet after the blooming.
Fig. 4 is a diagram showing one example of observation results of macro-photographs of the cross section of the billet.
Fig. 5 is a diagram showing relationship between a rate of incidence of defects on a surface of a billet that uses a test sample A and a thickness of scale of the steel ingot
Fig. 6 is a diagram showing relationship between a rate of incidence of defects of a surface of a billet that similarly uses a test sample B and a thickness of scale on the steel ingot.
Fig. 7 is a diagram showing relationship between a rate of incidence of defects of a surface of a billet that similarly uses a test sample C and a thickness of scale of the steel ingot.
Fig. 8 is a diagram showing relationship between a thickness of scale of the steel ingot and a holding temperature when an amount of steam in an atmosphere of a heating furnace is varied.

### BEST MODE FOR CARRYING OUT THE INVENTION

In a Fe-Cr alloy billet used in the present invention, a high reduction rate surface thereof may be covered with a scale layer at an area rate of 70 %, 80 %, 90 % or more. In other words, it may be covered with the scale layer at a total area rate of 35 % or more, 40 % or more or 45 % or more.

As shown in the examples described later, in the case of the high reduction rate surface being covered with the scale layer at an area rate of 70 % or more, the surface treatment rate can be reduced by substantially 50 % in comparison with comparative examples where descaling is applied.

In the Fe-Cr alloy billet used in the invention, there is tendency that the higher the area rate for the high reduction rate surface is, the lower the surface treatment rate of the billet is. For instance, in the case of the high reduction rate surface being covered with a scale layer at an area rate of 80 % or more, the treatment rate becomes substantially 30 % of that of a comparative example, and similarly in the case of being covered with a scale layer at an area rate of 90 % or more, the treatment rate becomes substantially 20 % of that of the comparative example. Accordingly, the area rate of the high reduction rate surface covered by the scale correlates well with the rate of incidence of defects on a surface of the billet.

In the manufacturing method according to the invention, in the blooming of the steel ingot, in order to remove scales generated during heating of the steel ingot, descaling with a high pressure water descaler is not applied. The reason for this is that as mentioned above, since a technology for completely removing the scale has not yet been established, it is intended to avoid a situation in which the scale remains incompletely or irregularly and is squeezed in and rolled together to cause a scale flaw.

In the manufacturing method according to the invention, although whether the blooming of the steel ingot is started from a high reduction rate surface or from a low reduction rate surface is not speculated, it is preferably started from the high reduction rate surface of the steel ingot. This is because when the high reduction rate surface is rolled at the first pass of the blooming, the scale generated on the steel ingot can be press-bonded sufficiently onto the high reduction rate surface.

Furthermore, a reason for press-bonding the scale onto the high reduction rate surface is because when the scale is squeezed in the high reduction rate surface with the scale insufficiently remained, the scale flaw is likely to be caused. In the invention, when the scale is closely attached at the area rate of 70 % or more, in a process of the blooming after that, the scale becomes unlikely to be squeezed in a matrix of the steel ingot. The tendency becomes more remarkable as the higher the area rate with which the scale covers becomes higher.

In a manufacturing method according to the invention, the scale having a thickness of 1000 µm or more that becomes a defect with difficulty in the blooming and is unlikely in causing a defect on the surface of the billet after the manufacture is generated on the steel ingot. The thickness of the scale can be obtained by controlling heating conditions (atmosphere, heating temperature and holding time) of the steel ingot.

Figs. 5 through 7 are diagrams showing relationship, in the case of the descaling being not applied, between the rate of incidence of defects on a surface of a Fe-Cr alloy billet and a thickness of the scale of the steel ingot. As test samples, 5 to 17 % Cr-containing alloys A, B and C shown in Table 1 are used. Fig.5 shows relationship with test sample A, Fig. 6 showing relationship with test sample B, and Fig. 7 showing relationship with test sample C, respectively

**Table 1**

| Test sample | Content of chemical component (mass %) | | | | | | | | |
|---|---|---|---|---|---|---|---|---|---|
| | C | Si | Mn | P | S | Cr | Ni | Mo | Fe |
| A | 0.18 | 0.25 | 0.5 | 0.015 | 0.007 | 5.0 | - | - | Bal. |
| B | 0.18 | 0.25 | 0.5 | 0.015 | 0.008 | 13.0 | - | - | Bal. |
| C | 0.18 | 0.25 | 0.5 | 0.014 | 0.008 | 17.0 | - | - | Bal. |

As specific conditions, test samples A, B and C are heated at a temperature of 1200 °C in an air atmosphere heating furnace with a holding time varied to alter the thicknesses of high reduction rate surface and a low reduction rate surface of the steel ingot. The test samples each are measured for the rate of incidence of defects on a surface of the billet. The reason for the air atmosphere heating furnace being set at a temperature of 1200 °C is due to the fact that the heating temperature is appropriate for reducing the deformation resistance in the blooming.

Furthermore, the measurement of the rate of incidence of defects on the surface of the billet is carried out by detecting the surface defects, after removing the scale on the billet surface by means of shot blasting, by use of a flaw detecting method with a leak detector of magnetic flux. The rate of incidence of defects is expressed in terms of a number ratio (number of billets where defects are detected/total billets number).

From results shown in Figs. 5 through 7, it is found that as the scale becomes thicker, the rate of incidence of defects decreases. When the thickness of the scale of the high reduction rate surface is 1000 µm or more, the rate of incidence of defects becomes 35 % or less, and furthermore when it is 1200 µm or more, the rate of incidence of defects becomes 25 % or less. The results, as explained in examples described later, show that the rate of incidence of defects is reduced to one half, furthermore substantially to one third that of the comparative example that is reproduced by a conventional method.

From this, in the invention, before blooming, the thickness of the scale on the steel ingot is preferably 1000 µm or more, and furthermore desirably 1200 µm or more.

A detail of the mechanism is not clear; however, it is assumed that when the rate of incidence of defects on the billet surface is intended to be suppressed, in order to cover the billet surface stretched by blooming with a scale layer having an area rate as large as possible, it is effective to secure a certain amount of scale, that is, a certain scale thickness.

Fig. 8 is a diagram showing the relationship between the thickness of the scale on the steel ingot and a holding temperature when the amount of steam in the atmosphere of a heating furnace is varied. In the drawing, the amount of steam contained in the atmosphere gas was varied as 0, 2.5, 10 and 20 % by volume %.

With 13 % Cr-containing alloy B shown in Table 1 as a test sample and with an atmosphere gas of 10 % CO₂-5 % O₂-Bal. N₂ as a basis, the concentration of steam contained in the atmosphere gas was varied in the range of 0 to 20 %. At this time, the steel ingot was heated at a temperature of 1200 °C and the holding time was varied, and the thickness of the scale generated on the steel ingot was measured.

The thickness of the scale was measured as follows: after the steel ingot was oxidized at a holding time of between 1 to 6 hr, a test sample was cut and then processed to a micro-sample and subsequently a cross section was observed. Furthermore, scale structures at this time are shown in Table 2.

From results shown in Fig. 8, in order to obtain a scale having a thickness of 1000 µm or more in an atmosphere that does not contain steam, heating of substantially 6 hr is necessary. The atmosphere that does not contain steam is substantially the same as air atmosphere.

On the other hand, by allowing containing 2.5 % or more of steam in the atmosphere, an oxidation speed can be very much improved. In order to effectively obtain a thickness of 1200 µm or more, in an atmosphere containing 2.5 % or more of steam, the steel ingot has only to be held for 2 hr or more at a temperature of 1200 °C.

**Table 2**

| Steam in atmosphere (%) | Structure of scale | |
|---|---|---|
| | External layer scale | Internal layer scale |
| 0 | Fe₂O₃ | FeCr₂O₄ |
| (not containing) | Fe₃O₄ | Fe₃O₄ |
| | Fe₂O₃ | FeCr₂O₄ |
| 2.5 to 20 | Fe₃O₄ | FeO |
| | FeO | |

As shown in Table 2, scale structures of all are constituted of two-layered structure including an external layer scale and an internal layer scale. In the invention, the external layer scale is a scale generated outside of a surface of an original steel strip and the internal layer scale is a scale generated inside of the surface of the original steel ingot.

In a scale formed in an atmosphere that contains 2.5 % or more of steam, the external layer scale is made of Fe₂O₃, Fe₃O₄ and FeO and the internal layer scale is made of FeCr₂O₄ and FeO. On the other hand, in a scale generated in an atmosphere that does not contain steam, the external layer scale is made of Fe₂O₃ and Fe₃O₄ and the internal layer scale is made of FeCr₂O₄ and Fe₃O₄.

Although the scale structure may be any of the above modes, as a scale structure that the scale defect cannot generate more easily, ones containing FeO are preferable. This is because, owing to high deformability of FeO itself, the FeO is not likely to cause destruction such as crack even under a large pressure, and furthermore, since the high temperature hardness thereof is lower than that of the steel ingot, the squeezing flaw is not likely to be caused.

For instance, Fe₂O₃ is hardly deformed, and furthermore, Fe₃O₄, when it is deformed by stretching experimentally at a very low speed at a temperature of 800 °C or more, can be stretched but cannot cope with a deformation speed during the rolling, resulting in causing crack and peeling off. On the other hand, FeO can deform in conformity with a deformation speed during the rolling and does not cause crack.

In the case of FeO being present, FeO is preferably contained 30 % or more as a thickness in the external layer scale when a cross section is subjected to micro-observation. The thickness of FeO can be measured by observing a color tone by means of the cross section micro-observation, by mapping O₂ (oxygen) by use of EPMA or by identifying in advance a structure of the whole scale by use of X-ray diffraction.

Furthermore, when the steam concentration becomes more than 20 %, effects of a rise of the scale generation speed and an increase in FeO ratio are gradually saturated. Accordingly, in consideration of damage of a furnace wall and the like of the heating furnace, the upper limit of the steam concentration is desirably set at substantially 25 %.

In the invention, in order to secure a scale thickness on the steel ingot of 1000 µm or more, a heating temperature of the steel ingot is desirably set at 1200 °C or more. Furthermore, the heating temperature, from viewpoints not only of scale generation but also of processability during the blooming, is desirably set at 1200 °C or more. On the other hand, the upper limit of the heating temperature, similarly, in consideration of the damage and the like of the equipment, is desirably set at 1300 °C or less.

In the invention, in order to secure a scale thickness on the steel ingot of 1000 µm or more, in the case of the heating temperature of the steel ingot being set at 1200 °C or more, the holding time is preferably set at 2 hr or more.

### (Example 1)

Effects exhibited by the manufacturing method of the present invention will be explained with reference to specific Example 1 and Example 2. Test materials were 5 to 17 % Cr-containing alloys A, B and C, and as a steel ingot starting material, a bloom CC material having a short side of 280 mm x long side of 600 mm x length of 7400 mm was used. The steel ingot was subjected to heating at 1200 °C for 6 hr in an atmospheric heating furnace (not containing steam). Furthermore, after heating the steel ingot, the manufacture was carried out under two conditions, that is, in one, descaling was applied with a high-pressure water descaler having a pressure of 100 kg/cm² and in the other, descaling was not applied.

The blooming of the steel ingot was performed at the first and second stand respectively by reverse rolling. The first pass of the rolling at the first stand was differentiated by whether the high reduction rate surface was reduced or the low reduction rate surface was reduced. Thereafter, at the first stand, the steel ingot was reduced to a cross sectional shape of substantially short side of 250 mm × long side of 400 mm, followed by finishing, at the second stand, into a billet of a final size of a diameter of 225 Ø.

After the billet was manufactured, surface scale was removed by shot blasting and flaw detection was performed by use of an NDI flaw detector due to magnetic leakage flux flaw detecting method. Here, flaws having a depth of 0.5 mm or more were detected. The flaw having a depth of 0.5 mm or more, when subjected to rolling and tubing as it is without treating, becomes a flaw on a surface of a steel tube; accordingly, it is necessary to treat a surface. A criterion was not determined on a length of defect. However, in consideration of being stretched to a final product, a defect having a small length such as several tens millimeters was checked.

The rate of incidence of defects was evaluated in terms of number ratio (number of generated defects/total number). At the last, an area rate with which the scale covers a surface of the billet was investigated. The area rate of the scale was measured in such a manner that a cross section observation sample was sampled from the high reduction rate surface of the billet for each 1 m, a length of peeled scale was observed by micro-observation, and {(average length of peeled scale in a vertical direction × average length of peeled scale in a horizontal direction) / total area} was calculated as an area rate. As the area rate of the scale, an average value of the area rates of all samples in the respective billets was used.

The frequencies of incidence of defects and the area rates of scales that cover the high reduction rate surface of the billet at this time are shown in Tables 3 through 5. Table 3 shows results of 5 % Cr-containing alloy A was used as a test sample; Table 4 shows results of 13 % Cr-containing alloy B was used as a test sample; and Table 5 shows results of 17 % Cr-containing alloy C was used as a test sample.

In Example 1, in each case where any of the test samples was used, thicknesses of scales formed on steel ingots immediately after taking out of a heating furnace were substantially 1000 µm, and the scale structure was made of an external layer scale of Fe₂O₃ and Fe₃O₄ and an internal layer scale of FeCr₂O₄ and Fe₃O₄. Furthermore, thicknesses of scales covering surfaces of the billets immediately after the manufacture were 150 µm or more.

**Table 3**

| Test No. | Blooming | | State of billet | | | Group |
|---|---|---|---|---|---|---|
| | Descaling | Rolled surface at the first pass | Rate of incidence of defects (%) | Scale area rate (%) | | |
| | | | | High reduction rate surface | All surface of billet | |
| A1 | Applied | Low reduction rate surface | 92 | 50 | 25 | Comparative example |
| A2 | Applied | High reduction rate surface | 97 | 48 | 24 | |
| A3 | Not applied | Low reduction rate surface | 47 | 73 | 36.5 | Inventive example |
| A4 | Not applied | High reduction rate surface | 35 | 83 | 41.5 | |

| | | | | | | |
|---|---|---|---|---|---|---|
| Note) Test sample: 5 % Cr-containing alloy A | | | | | | |

**Table 4**

| Test No. | Blooming | | State of billet | | | Group |
|---|---|---|---|---|---|---|
| | Descaling | Rolled surface at the first pass | Rate of incidence of defects (%) | Scale area rate (%) | | |
| | | | | High reduction rate surface | All surface of billet | |
| B1 | Applied | Low reduction rate surface | 97 | 49 | 24.5 | Comparative example |
| B2 | Applied | High reduction rate surface | 93 | 47 | 23.5 | |
| B3 | Not applied | Low reduction rate surface | 45 | 71 | 35.5 | Inventive example |
| B4 | Not applied | High reduction rate surface | 33 | 82 | 41 | |

| | | | | | | |
|---|---|---|---|---|---|---|
| Note) Test sample: 13 % Cr-containing alloy B | | | | | | |

**Table 5**

| Test No. | Blooming | | State of billet | | | Group |
|---|---|---|---|---|---|---|
| | Descaling | Rolled surface at the first pass | Rate of incidence of defects (%) | Scale area rate (%) | | |
| | | | | High reduction rate surface | All surface of billet | |
| C1 | Applied | Low reduction rate surface | 94 | 50 | 25 | Comparative example |
| C2 | Applied | High reduction rate surface | 98 | 45 | 22.5 | |
| C3 | Not applied | Low reduction rate surface | 44 | 70 | 35 | Inventive example |
| C4 | Not applied | High reduction rate surface | 32 | 80 | 40 | |

| | | | | | | |
|---|---|---|---|---|---|---|
| Note) Test sample: 17 % Cr-containing alloy C | | | | | | |

As shown in Tables 3 through 5, in the case of the descaling being applied in the blooming as comparative examples, the scale coverage was in the range of 45 to 50 % by the area rate of the high reduction rate surface (22.5 to 25 % in terms of the total area), the rate of incidence of defects was nearly the total number, and with the number rate of 92 to 98 % surface treatment was necessary

On the other hand, in the case of, among the inventive examples, the low reduction rate surface being rolled in the first pass, the scale coverage of the high reduction rate surface was such high as in the range of 70 to 73 % by the area rate of the high reduction rate surface (35 to 36.5 % in terms of the total area), the rate of incidence of defects were dropped as much as 44 to 47 %. That is, one half that of the comparative examples. Furthermore, when the high reduction rate surfaces were rolled at the first pass in the inventive examples, the scale coverage was such high as in the range of 80 to 83 % in the area rate of the high reduction rate surface (40 to 41.5 % in terms of the total area), and at the same time, the rate of incidence of defects was reduced to substantially one third that of the comparative examples, that is, 32 to 35 %.

From results shown in Tables 3 through 5, it is found that when the scale coverage is substantially 70 % (35 % in terms of total area rate) in the area rate of the high reduction rate surface, the rate of incidence of defects is reduced to substantially 50 % compared to the comparative example where the descaling is applied, and furthermore, when the scale coverage is substantially 80 % (40 % in terms of total area rate) in the area rate of the high reduction rate surface, the rate of incidence of defects is reduced to substantially one third compared to that of the comparative example.

This is assumed that although a detail of the mechanism is not clear, when the scale is adhered with a certain area rate close to an entire area or more, uneven scales that cause indentations or inclusions can be inhibited from occurring.

### (Example 2)

Steel ingots obtained with test samples and steel strip of starting materials under the same conditions as example 1 were heated in a heating furnace. At this time, a moistening device was connected to the atmospheric furnace to vary an atmosphere in the furnace, and heating was carried out at 1200 °C for 6 hr.

The conditions of the blooming after the heating and measurement conditions of the rate of incidence of defects and area rate with which scales cover after the manufacture of billets were set as the same as that of (Example 1), and thereby an influence that the heating atmosphere affects on the rate of incidence of defects of the billet was investigated. Results of investigation are shown in Tables 6 through 8.

In results of investigation, Table 6 shows results when 5 % Cr-containing alloy A was used as a test sample, Table 7 shows results when 13 % Cr-containing alloy B was used as a test sample, and Table 8 shows results when 17 % Cr-containing alloy A was used as a test sample. In each of cases where the above test samples were used in Example 2, a thickness of the scale that covers the surface of the billet was 150 µm or more.

As shown in Tables 6 through 8, it is found that in the inventive examples, as the concentration of steam in the atmosphere increases, the area rate with which the scale covers the high reduction rate surface increases and at the same time the rate of incidence of defects of the billet decreases. This is because a content of steam increases, the scale grows thicker on the steel ingot and at the same time FeO that is unlikely to be squeezed in a mother material during the blooming is much generated.

Among the inventive examples that use the respective test samples, as shown in test Nos. A8 and A9, B8 and B9 and C8 and C9, when the steel ingot before blooming was held in an atmosphere containing 10 % or more of steam at a heating temperature of 1200 °C or more for 2 hr or more to generate the scale, the area rate of the high reduction rate surface that the scale covers can be increased to 93 % or more, and the rate of incidence of defects of the billet can be reduced to 22 % or less.

### INDUSTRIAL APPLICABILITY

According to the manufacturing method of the present invention, since blooming is carried out with the high reduction rate surface of the steel ingot covered with a scale layer having a large area rate, the indentation and inclusion of the scale can be reduced. Thereby, in the case of a billet for use in seamless steel pipes being manufactured from a steel ingot of a Fe-Cr alloy, surface treatment before tube-making can be largely reduced.

Accordingly, in the method of manufacturing seamless steel pipes according to the invention, even when making Fe-Cr alloy steel pipe which is relatively hard to process, the pipes can be manufactured at low manufacturing costs and efficiently, and the method can be widely applied in the field of manufacturing hot seamless steel pipes.

## Claims

1. A method of manufacturing a seamless steel pipe, comprising subjecting a steel ingot (1) to blooming to manufacture an Fe-Cr alloy billet (2), wherein the ingot is heated prior to blooming to generate a scale on its surface and wherein blooming is applied without applying descaling of the steel ingot, and manufacturing the seamless steel pipe from the Fe-Cr alloy billet (2).

2. A method according to claim 1, wherein a scale having a thickness of 1000 µm or more is generated on the steel ingot.

3. A method according to claim 2, wherein a high reduction rate surface (3) of the steel ingot is reduced first.

4. A method according to claim 2 or 3, wherein the steel ingot is held in an atmosphere containing 2.5 % or more of steam, by volume %, at a heating temperature of 1200 °C or more for 2 hr or more to generate the scale.

## Patentansprüche

1. Verfahren zum Herstellen eines nahtlosen Stahlrohrs, welches das Unterziehen eines Stahlrohblocks (1) einem Vorblocken, um einen Knüppel (2) aus Fe-Cr-Legierung herzustellen, wobei der Rohblock vor dem Vorblocken erwärmt wird, um auf dessen Oberfläche einen Zunder zu erzeugen, und wobei das Vorblocken ohne Durchführen von Entzundern des Stahlrohblocks durchgeführt wird, und Herstellen des nahtlosen Stahlrohrs aus dem Knüppel (2) aus Fe-Cr-Legierung umfasst.

2. Verfahren nach Anspruch 1, wobei ein Zunder mit einer Dicke von 1000 µm oder mehr auf dem Stahlrohblock erzeugt wird.

3. Verfahren nach Anspruch 2, wobei eine Oberfläche (3) hoher Reduktionsrate des Stahlrohblocks zuerst reduziert wird.

4. Verfahren nach Anspruch 2 oder 3, wobei der Stahlrohblock 2 Stunden oder länger in einer nach Volumenprozent 2,5% oder mehr Dampf enthaltenden Atmosphäre bei einer Erwärmungstemperatur von 1200 °C oder mehr gehalten wird, um den Zunder zu erzeugen.

## Revendications

1. Procédé de fabrication d'un tuyau en acier sans raccord, comprenant la soumission d'un lingot d'acier (1) à une efflorescence pour fabriquer une billette d'alliage Fe.Cr (2), dans lequel le lingot est chauffé avant l'efflorescence pour générer une calamine sur sa surface et dans lequel l'efflorescence est appliquée sans appliquer un décalaminage du lingot d'acier, et la fabrication du tuyau en acier sans raccord à partir de la billette d'alliage Fe.Cr (2).

2. Procédé selon la revendication 1, dans lequel une calamine ayant une épaisseur de 1000 µm ou plus est générée sur le lingot d'acier.

3. Procédé selon la revendication 2, dans lequel une surface à taux de réduction élevé (3) du lingot d'acier est réduit dans un premier temps.

4. Procédé selon la revendication 2 ou 3, dans lequel le lingot d'acier est maintenu dans une atmosphère contenant 2,5 % ou plus de vapeur, en % en volume à une température de chauffage de 1200 °C ou plus pendant 2 h ou plus pour générer la calamine.
